

# UNITED STATES PATENT OFFICE.

KENNETH L. BINKLEY, OF NEW YORK, N. Y., ASSIGNOR TO THE BARRETT COMPANY.  
A CORPORATION OF NEW JERSEY.

## PLASTIC COMPOSITION.

1,418,905.

Specification of Letters Patent. Patented June 6, 1922.

No Drawing.

Application filed November 29, 1920. Serial No. 427,019.

To all whom it may concern:

Be it known that I, KENNETH L. BINKLEY, a citizen of the United States, residing at 100 Lexington Avenue, New York, in the county of New York and State of New York, have invented certain new and useful Improvements in Plastic Compositions, of which the following is a specification.

This invention relates to a material that is plastic when hot, which material is especially adapted for roofing purposes. It relates more particularly to the production of a composition of matter containing a relatively low melting point pitch mixed with a filler which will so modify the pitch as to render the same suitable for roofing purposes and which may be satisfactorily used even on steep roofs without sliding.

Many materials have been tried, such as pitch or asphalt mixed with different sorts of inorganic fillers, but difficulties have been encountered with these substances, due to the fact that some of the fillers would be injured when the pitch or asphalt was heated to be applied to the roof; or the fillers would deleteriously affect the pitch or asphalt; or the fillers would not remain permanently suspended in pitch or asphalt.

At present the pitches that are used for roofing purposes, do not stand up satisfactorily, on inclines more than two inches to the foot. The heat, particularly in the summer, from the direct rays of the sun and from other sources causes the pitch to run and slide. This running and sliding of the pitch defeats the very purpose for which it was intended.

A pitch to be entirely satisfactory for steep roofing purposes should, when heated, be easily mopped, hold heat, have elasticity and adhesiveness, heal with the rays of the sun, should it develop cracks due to expansion or contraction because of weather conditions, and be of such a consistency that it will not slide or run in hot weather on any normal roof inclines, and my invention meets all these requirements.

A straight pitch of low melting point will not fill the demand and neither will straight pitch of a high melting point, but I have found that a composition of matter comprising pitch and magnesium carbonate will give the desired results.

By the present invention, using mag-

nesium carbonate, I have produced a composition in which this filler will withstand, without injury, a temperature as great as that to which the pitch itself is subjected during its application to a roof. The filler is also very finely subdivided so that when mixed with the pitch, a composition is produced which has the characteristic of being smooth. At the same time the filler has good suspension qualities, so that the danger of the same settling out of the melted pitch during application is practically eliminated. The filler does not have any chemical action on pitch, nor does it produce other deleterious influences upon it. At the same time the filler mixed with the pitch produces a composition which is workable at a lower temperature, namely about 350° F. to 500° F., than has been usual with the asphalt or pitches heretofore used for steep roofing purposes. The composition thus produced seems to be self-healing. That is, if when cold it becomes accidentally cracked, the cracks subsequently mend on warming so as to produce again a continuous sheet. When spread out it is smooth and will maintain a high gloss and sheen, and at the same time will not slide or run to an appreciable extent, even when exposed to the direct rays of the sun in the hottest climates. This composition also has the advantage over present roofing pitches or compositions in that it holds heat for a much longer period and is, therefore, easier of application.

In practicing this invention I mix pitch with a certain percentage of magnesium-carbonate, thereby producing a composition of matter which has a higher melting point than the pitch but at the same time the composition can be rendered plastic by the application of sufficient heat, so that the same is capable of being applied to a roof by means of a mop.

As a specific illustration of my invention I will give the following proportions, but it is to be understood that this is merely illustrative of the invention as the proportions and melting point of the pitch may be varied over a wide range without departing from the spirit or scope of this invention.

I take coal tar pitch of a melting point of about 160° F. (determined by the cube in 110

water method) and containing about 25% of free carbon. This is mixed with about one-ninth as much by weight of magnesium carbonate. The mixture is heated and 5 stirred so that the magnesium carbonate becomes well distributed throughout the mass. The melting point of the finished product is thereby increased to about 208° F.

Particles of pitch of the proper melting 10 point can be mixed with magnesium carbonate and the mixture dumped into an agitating still and heated to the proper temperature; or coal tar can be distilled until the residuum is a pitch of the proper melting 15 point, whereupon the magnesium carbonate may be introduced into the molten pitch; or coal tar and the proper amount of magnesium carbonate can be mixed together and placed in a still where the proper 20 amount of volatile constituents are distilled off, leaving a residue of the proper melting point. It is clear that, irrespective of the method employed, it is desirable to ob-

tain a composition which contains pitch and magnesium carbonate, as this composition 25 possesses the desirable characteristics for roofing purposes. When I speak of magnesium carbonate I mean to include the basic carbonates of magnesia which are ordinarily found as commercial products and in no 30 way desire to limit myself to normal carbonates of magnesia.

I claim:

1. A composition of matter comprising pitch and magnesium carbonate, said composition having a melting point of about 35 200° F.

2. A composition of matter comprising pitch of a melting point of about 160° F. and magnesium carbonate. 40

3. A composition of matter comprising pitch and magnesium carbonate in substantially the proportions of 9 to 1 by weight.

In testimony whereof I affix my signature.

KENNETH L. BINKLEY.